

April 9, 1935.

N. B. ORNITZ

1,997,469

FURNACE ROLL AND THE LIKE

Filed April 5, 1933



INVENTOR

Nathaniel B. Ornitz  
Byrnes, Stebbins, Parmelee & Blenko  
his attorneys

## UNITED STATES PATENT OFFICE

1,997,469

## FURNACE ROLL AND THE LIKE

Nathaniel B. Ornitz, Pittsburgh, Pa.

Application April 5, 1933, Serial No. 664,520

## 1 Claim. (Cl. 263—6)

The present invention relates to furnace parts, such as rolls and skids, which are intended for use under exposure to furnace gases at high temperature. More particularly, my invention relates to furnace parts formed of a chromium-nickel ferrous alloy having the nickel, chromium and other elements of such absolute and relative proportions that there is imparted to such furnace parts a remarkable structural strength, resistance to abrasion and resistance to corrosive attack of sulphurous gases at high temperatures.

There has been a demand for furnace parts, such as rolls and skids, which have high resistance to abrasion, resistance to corrosive attack of sulphurous gases, and structural strength at high temperatures, such furnace parts being in particular demand for annealing and normalizing furnaces, where the parts must have a high temperature so as not to cool the sheets or other articles being annealed or normalized. The temperatures at which such parts should operate are frequently as high as about 2000° F. Such furnaces are frequently fired with gases containing sulphurous compounds, and to resist such gases, it is necessary that the furnace parts resist the corrosive action of the sulphur compounds even at these elevated temperatures. The parts which support the materials being heat treated, such for example, as the rolls or skids in an annealing or normalizing furnace, are subject to abrasion, and it is necessary that the material have a high resistance to abrasion at the elevated temperatures employed.

Examples of such parts are shown in the drawing in which,

Fig. 1 is illustrative of a roll adapted to be used in an annealing or normalizing furnace, and

Figs. 2 and 3 are respectively a plan view and a view in side elevation of a skid adapted to be used in such furnaces.

The roll shown in Fig. 1 is merely one example of a great many different types of furnace rolls to which my invention may be applied. This roll comprises a shaft 4 and a plurality of discs 5 upon which the sheets or the like may travel.

The skid 1 shown in Figs. 2 and 3 is provided with lugs 8 engageable with suitable supports such as the hollow rods 9.

I have succeeded in producing rolls, skids and other furnace parts which meet the exacting conditions present in furnaces of the type mentioned above, wherein such parts are called upon to resist gases containing sulphurous compounds and in which the temperature frequently rises as high or higher than 2000° F. Such furnace parts

successfully meet all of the conditions required when I have formed them of a chromium-nickel ferrous alloy having the nickel, chromium, and other elements restricted within certain narrow ranges of proportions.

The base of my alloy is iron usually supplied as low carbon steel scrap. The alloy is preferably melted in an electric furnace since this gives good control of the alloying elements and the carbon.

The chromium in my alloy may vary from about 27 to 35%, preferably from 27.5 to 32%, and in the preferred specific formula, I use chromium from 28 to 32%. The nickel may vary from about 4 to 11%, preferably between 6 to 11%, and in the preferred specific formula, the nickel is held to between 6 to 8%. The silicon may vary in accordance with good steel-making practice, say between about .15 to 3%, but preferably between 1 to 2%. In the preferred specific formula, the silicon is about 1½%. The manganese may have the usual variations in steel-making practice, say between about .30 to 2%, but preferably between .50 to 1%, and in the preferred specific formula, the manganese is about .60%.

The carbon should be kept as low as practicable. The lower the carbon, the better the heat-resisting properties of the alloy. For good results, the carbon should not be over about 1%, preferably not over .60%, and in the specific formula employed, the carbon is not over .30%.

The sulphur and phosphorus are kept as low as practicable by suitable selection of the raw materials. I prefer that the sulphur shall not be over about .10%, and in my preferred formula, the sulphur is not over .05%. Similarly, I prefer that the phosphorus shall not be over about .10%, and in my preferred formula not over .04%.

The raw material such as the low carbon steel scrap, the low carbon ferro-chromium and the metallic nickel, are charged and melted in an electric furnace in the usual way, and the charge tapped out into castings or ingots as required.

Small amounts of other alloying elements may be used, such for example, as tungsten, cobalt, vanadium, titanium, aluminum, etc., which, when present in relatively minor quantities, do not materially affect the heat-resisting properties of the alloy.

Articles made from my alloy, either cast, forged or rolled, have a novel combination of desirable properties which particularly adapt them for high temperature furnace work. Parts made from this alloy have a remarkable struc-

tural strength and hardness at high temperatures, say 1700 to 1900° F. The parts so made are adapted for those uses which require structural strength and resistance to abrasion, such 5 for example, as the rolls which support and feed sheets or other articles through an annealing or normalizing furnace.

According to my best observations and tests which I have at the present time, furnace parts 10 made of an alloy such as the one disclosed as my preferred formula actually grow harder as the temperature is increased above 1500° F., reaching its maximum high temperature hardness at 1850° F. After this there is a gradual 15 softening, although the parts retain good structural strength and hardness even at 2000° F. Normalizing furnace rolls of my alloy have been successfully operated at temperatures as high as 2000° F., and may be used under no load conditions 20 at temperatures as high as 2100° F.

The furnace parts made of this alloy have not only remarkable hardness and structural strength as ordinarily measured, but also have a remarkable resistance to the so-called creep or slow flow 25 which causes ultimate failure of furnace parts at high temperatures under long continued 30 stresses,

At the furnace temperatures frequently employed in annealing and normalizing furnaces, 30 say at 1700 to 2000° F., furnace parts made of my alloy have a remarkable resistance to the corrosive action of the sulphurous gases which are present in the gaseous products of combustion from sulphur-containing fuel, such for example, 35 as producer gas, blast furnace gas or coke oven gas. There is practically no scaling or disintegration or deterioration of the furnace parts under the action of such gases.

I have found that the optimum results have 40 been obtained in making articles such as rolls, roll shafts, and roll disks for annealing and normalizing furnaces using an alloy having the preferred formula set forth above, although certain variations may be made in it as above indicated. 45 There are, however, rather narrow limits to the variations in the nickel and chromium contents. If the nickel is materially increased above 11%, the alloy is attacked by the sulphurous gases at high temperatures. Indeed, if the conditions are 50 particularly rigorous as regards sulphur content and temperature of the furnace gases, the nickel should not be substantially above 8%. If the nickel is lowered below my proportions, the structural strength, hardness and creep or flow point 55 are decreased so that the material will not stand up under the high temperatures employed in the modern annealing and normalizing furnaces.

If the chromium is decreased below my proportions, the chromium ceases to offer effective protection to the nickel and the alloy is attacked 60 by the sulphurous gases as well as by oxygen at

high temperatures. As the chromium content is lowered, its effectiveness in resisting the sulphurous and oxidizing gases decreases as the carbon content increases, so that unless the carbon content is held low, the chromium cannot be lowered much below that of the preferred proportions; although if the carbon content is held low, there is a little more latitude in decreasing the chromium content. If the chromium content is higher than my proportions, there is a 10 tendency to objectionable brittleness and the cost is unnecessarily increased since low carbon ferro-chromium is expensive.

As above pointed out, my invention relates particularly to articles requiring structural strength, resistance to abrasion and resistance to corrosion at high temperatures, and especially to furnace parts, such for example, as rolls, roll disks, roll shafts, skids and other furnace parts, which must be maintained at a high temperature 15 so as not to chill the articles which are carried thereby, such for example, as the sheets in a sheet annealing or normalizing furnace.

Rolls of my annealing or normalizing furnace may be maintained continuously at temperatures 25 in the neighborhood of 1700 to 2000° F., which are the temperatures of the furnace gases. My rolls under such conditions have been continuously 30 and successfully employed for a considerable period of time without failure, whereas the rolls made of the best of the other alloys heretofore known for such purposes have failed under the severe furnace conditions. The furnace referred to was a continuous pack-heating furnace in which the rolls had to be operated at a temperature of 1900° F. and where the producer gas used 35 was made from a coal containing about 3% of sulphur.

This application is a continuation-in-part of my copending application Ser. No. 359,428, filed 40 April 30, 1929.

While I have specifically described the preferred embodiment of my invention and the characteristics of the articles made from my alloy, it is to be understood that the invention is not so limited, but may be otherwise embodied and practiced within the scope of the following claim.

I claim:

A roll for a high temperature annealing or normalizing furnace formed of a ferrous alloy containing chromium about 28% to 32%, nickel about 50 6% to 8%, silicon about 1% to 2%, manganese about .5% to 1%, carbon not over about .30%, sulphur not over about .05%, and phosphorous not over about .04%, the balance of the alloy 55 being substantially iron, and characterized by its structural strength, resistance to abrasion and resistance to corrosion by the furnace gases at high temperatures.

NATHANIEL B. ORNITZ.